

Jan. 11, 1972

E. C. EVANS

3,634,259

CLEANSING LOTION FOR PERSONAL HYGIENE

Filed Feb. 24, 1969

2 Sheets-Sheet 1



Figure 1

Jan. 11, 1972

E. C. EVANS

3,634,259

CLEANSING LOTION FOR PERSONAL HYGIENE

Filed Feb. 24, 1969

2 Sheets-Sheet 2



Figure 2

1

3,634,259

CLEANSING LOTION FOR PERSONAL HYGIENE  
Ernest C. Evans, Appleton, Wis., assignor to Kimberly-Clark Corporation, Neenah, Wis.  
Filed Feb. 24, 1969, Ser. No. 801,272  
Int. Cl. C11d 1/00

U.S. Cl. 252—89

6 Claims

## ABSTRACT OF THE DISCLOSURE

A cleansing preparation in lotion-like form designed especially for personal hygiene and proctological use, characterized by a particular viscosity and horizontal wicking rate.

## BACKGROUND OF THE INVENTION

In practicing personal hygiene, there is a great need for a convenient means for cleansing the skin in the anal and perianal zones after defecation. In Europe, in many parts of South America, and in other scattered parts of the world, a flush basin known as the bidet is a standard bathroom fixture especially designed for this purpose, and is considered by physicians as a real advance in culture and in hygiene. Even though the United States manufactures and exports bidets, it must be said, unfortunately, that they are rarely found in the American home.

The present practice is to wipe the anal region with absorbent toilet paper after a bowel movement. While the absorbent paper is effective in removing the major portion of the feces it does not do an efficient job and tends to smear rather than cleanse. Vigorous rubbing also has an abrasive effect, no matter how soft the paper, and such rubbing frequently bruises sensitive tissues permitting bacteria to enter the broken anal and perianal skin areas whereby the body is more easily susceptible to infection.

While the majority of proctologists advice that water is by far the most effective cleansing agent for the purpose, it is unfortunate that water is not readily available in a convenient form in most lavatories other than as provided by the bidets mentioned above, and thus is not used for cleansing as commonly as it should be used for that purpose. This invention is directed to a means for providing an aqueous medium in a form which is readily adapted for cleansing use, and which may be supplied in suitable dispensing fixtures, or which may be carried by the user in a small squeeze bottle or the like.

## SUMMARY OF THE INVENTION

The present invention provides an aqueous solution of a water-soluble resin in an amount sufficient to increase the viscosity of the water up to a range which permits it to be deposited on absorbent toilet tissue without prematurely spreading out on the paper and/or penetrating therethrough. The solution also has a slow wicking rate which makes it capable of eventually wetting the tissue upon standing, or if pressure is applied in use. The solution has a lotion-like feel and appearance, and when it is applied to the skin it spreads easily and has a cool, soothing effect. This lotion-like solution is effective in cleansing the skin with one or more applications, and accomplishes this task without excessive wiping and accompanying abrasion. Any residual dampness after cleansing may be removed with lotion-free paper.

It is therefore the principal object of this invention to provide a cleansing lotion particularly adapted for personal hygiene and proctological use.

An additional object is to provide a cleansing lotion which may be applied to absorbent toilet tissue without

2

prematurely spreading out on the paper surface and/or penetrating therethrough.

Other objects and advantages of the invention will become apparent by reference to the following specification and accompanying drawings wherein there is described various selected embodiments of the invention.

## BRIEF DESCRIPTION OF THE DRAWINGS

FIG. 1 is a graph showing viscosities and wicking times of various solutions, including both desirable and undesirable types.

FIG. 2 is a schematic representation, partly in section, of a testing set-up used to measure the wicking time of the various solutions charted in FIG. 1.

## DESCRIPTION OF THE PREFERRED EMBODIMENTS

In making a preliminary research study directed toward finding suitable cleansing agents which might be capable of application to toilet paper for purposes of anal cleansing, it was found that most water-based liquids and lotions available on the market, and which might possibly be adapted for this purpose, were of such a nature that they either penetrated the absorbent paper so rapidly that the strength of the paper was destroyed and the paper ruptured easily and became useless for its intended purpose, or that they would not wet the paper or skin at all and thus were ineffective as cleansing agents. Oily or fatty-acid based liquids were also ineffective for similar reasons. It became apparent, therefore, that what was needed was a water-based material sufficiently viscous in nature to stay on the surface of absorbent paper and yet sufficiently fluid to spread easily when applied to the skin with the paper. After extensive studies involving many trials and errors it was found that the desired properties were provided by some aqueous solutions of particular water-soluble resins in amounts to provide a solution having a Brookfield LVF viscosity in the range of 2000 to 7000 centipoises measured at 20 r.p.m. with a No. 3 spindle. While some aqueous solutions in the above-noted viscosity range worked satisfactorily, it was found that more than viscosity was required to provide a suitable lotion. In other words, some materials which fell in the preferred viscosity range would not penetrate the paper at all, or wet the skin sufficiently to perform the cleansing function. After further study it was determined that wicking ability was a determining factor in providing these latter properties. It became apparent that a useful fluid should have the ability to penetrate absorbent paper, but that the rate of penetration should be slow and gradual.

After it was determined that wicking rate could be measured by using a standardized absorbent paper having carefully controlled porosity and measuring the speed at which the fluid being tested travels in the paper, a test was devised to measure wicking rate and establish operable ranges.

Suitable test equipment for this purpose is shown in FIG. 2. A horizontal plate 12 of clear acrylic plastic is provided, and has placed on its surface a strip of No. 1 Whatman Filter paper 13, cut  $\frac{1}{4}$ " wide. On top of this paper strip is placed a second or loading plate 14 of clear acrylic plastic, and a 500 gm. weight 15 is placed on top of plate 14. The total loading of the system is about 25 gms./sq. in.

A vessel 16 is completely filled with the fluid 17 to be tested and moved into position so that the top surface of the fluid touches the lower surface of plate 12 and so that at least the tip of the filter paper 13 is in contact with the fluid 17. The lower plate 12 is calibrated in tenths of inches, and the overhang of the paper is set at a predetermined length, in this case  $\frac{1}{2}$  inch, so that the progression of the wet column along the paper and plate may be noted

in measurable increments. Readings are taken every half minute of time lapse. The wetted column length in inches is plotted as a function of time in minutes. Results of a number of tests are shown in FIG. 1 where the slope of each plot is an indication of the speed of wicking. In general, as the viscosity of any particular solution is increased, the slope of the line decreases. It is noted that the wicking rate is not the same for different fluid compositions of the same viscosity.

By referring to the chart it will be noted that water alone, with a viscosity of 1, has the fastest wicking rate. A solution containing 0.15% of the ammonium salt of carboxypolymethylene (CPM) has a Brookfield viscosity of 500 centipoises and a wicking rate of about 0.1 inch per minute. A solution containing 0.19% CPM has a viscosity of 1000 cps. and a wicking rate of about 0.1 to about 0.06 inch per minute. Solutions containing 0.21% CPM to 0.26% CPM have viscosities ranging from 2000 cps. to 7000 cps. and wicking ranges of about .03" to about .05" per minute.

The ranges of viscosity and wicking rate in the latter group were found to provide lotions with the desired properties.

Liquids above this range wetted the paper too rapidly. Those below this range were too viscous and did not wet the paper or skin sufficiently to do an effective cleansing job.

Among the latter were solutions using various percentages of hydroxyethylcellulose (HEC) and carboxymethylcellulose (CMC). It will be noted from the FIG. 1 graph, that the solutions containing these latter two resins had very low wicking rates and most of them did not wick at all. Solutions containing 0.09%, 0.11%, and 0.15% HEC, respectively, had viscosities of 300, 1300 and 3000 centipoises, respectively, and did not wick at all, as indicated by the line coincident with the base line for time in minutes. A solution containing 4.0% CMC at 5000 cps. also did not wick. When the solution containing HEC was diluted still further to 0.03% HEC, the solution had a viscosity of 45 cps. and wicked only slightly.

From the above it will be noted that the only satisfactory solutions found were those containing the carboxypolymethylene resin. Carboxypolymethylene resins are well-known thickeners, and most commonly comprise carboxypolymethylene resin neutralized with ammonium hydroxide and used in the form of the ammonium salt. Other alkalis, such as sodium or potassium hydroxide may also be used.

While any of the concentrations in the useful ranges as set forth above may be used, a preferred formulation comprised 0.24% of the ammonium salt of carboxypolymethylene resin; 96.66% water; and 0.1% preservative, in the latter case hexachlorophene. This mixture had a viscosity of about 5000 cps. and a wicking rate of about .04" per minute. When deposited onto absorbent paper, this aqueous solution stood on the surface in globular form and did not soak through to any noticeable degree even after several minutes. When applied to the skin it had an agreeable cool feeling, and cleansed test areas adequately. Any surplus was easily removed with a dry sheet of paper.

While the alkali salt of carboxymethylene resin when used alone is sufficient to obtain the desired results, other ingredients may be added if desired. For example up to

5% of a lubricant such as glyceryl monostearate may be used. Cetyl alcohol is another satisfactory lubricant. These materials provide a smoother, easier to apply lotion which is sometimes desired. Addition of these materials tend to increase viscosity of the CPM solutions, but as long as the viscosity is controlled between 2000 and 7000 cps. the wicking rate remains in a satisfactory range. In addition, bactericidal agents such as the previously mentioned hexachlorophene, bithionol and the like may be used. For esthetic and cosmetic effects, coloring materials and fragrances may also be added.

10 It is also preferred that deionized water be used so that the desired viscosities may be more easily controlled.

15 While the above describes preferred embodiments of the invention various changes may be made without departing from the spirit thereof.

What is claimed is:

1. A cleansing lotion especially adapted for proctological use consisting essentially of an aqueous solution of a water-soluble resin, said resin being an alkali metal or ammonium salt of carboxypolymethylene and being present in the amount of from about 0.21% to about 0.26% by weight, said solution being characterized by a Brookfield LVF viscosity of between 2000 and 7000 centipoises measured with a No. 3 spindle at 20 r.p.m. and being further characterized by a horizontal wicking rate of from .03" to .05" per minute.

2. The lotion of claim 1 in which the aqueous medium is deionized water.

3. The lotion of claim 1 in which said alkali metal salt is selected from the group consisting of ammonium, potassium, and sodium salts.

4. The lotion of claim 3 in which said salt is the ammonium salt of carboxypolymethylene.

5. The lotion of claim 1 in which said solution also contains a lubricant selected from the group consisting of glyceryl monostearate and cetyl alcohol in an amount less than 5% by weight.

6. The lotion of claim 1 in which said solution also contains about 0.1% by weight of a preservative selected from the group consisting of hexachlorophene and bithionol.

#### References Cited

##### UNITED STATES PATENTS

|    |           |         |              |       |        |
|----|-----------|---------|--------------|-------|--------|
| 45 | 1,786,513 | 12/1930 | Zuckerman    | ----- | 252-91 |
|    | 2,798,053 | 7/1957  | Brown        | ----- | 252-91 |
|    | 2,999,265 | 9/1961  | Duane et al. | ----- | 252-91 |
|    | 3,011,950 | 12/1961 | Mehaffey     | ----- | 424-78 |

##### FOREIGN PATENTS

|       |      |               |       |           |
|-------|------|---------------|-------|-----------|
| 3,984 | 1874 | Great Britain | ----- | 15-104.93 |
|-------|------|---------------|-------|-----------|

##### OTHER REFERENCES

Carbopol, Chem. & Eng. News, Sept. 29, 1958, pp. 64-5.

LEON D. ROSDOL, Primary Examiner

W. E. SCHULZ, Assistant Examiner

60 U.S. Cl. X.R.

252-92; 424-78